



US008747643B2

(12) **United States Patent**  
**Niazimbetova et al.**

(10) **Patent No.:** **US 8,747,643 B2**  
(45) **Date of Patent:** **Jun. 10, 2014**

(54) **PLATING BATH AND METHOD**

(75) Inventors: **Zukhra I. Niazimbetova**, Westborough, MA (US); **Maria Anna Rzeznik**, Shrewsbury, MA (US)

(73) Assignee: **Rohm and Haas Electronic Materials LLC**, Marlborough, MA (US)

(\*) Notice: Subject to any disclaimer, the term of this patent is extended or adjusted under 35 U.S.C. 154(b) by 0 days.

(21) Appl. No.: **13/214,723**

(22) Filed: **Aug. 22, 2011**

(65) **Prior Publication Data**

US 2013/0048505 A1 Feb. 28, 2013

(51) **Int. Cl.**  
**C25D 3/38** (2006.01)  
**C23C 18/40** (2006.01)

(52) **U.S. Cl.**  
USPC ..... **205/296**; 205/297; 205/298; 106/1.26

(58) **Field of Classification Search**  
USPC ..... 106/1.26; 205/296, 297, 298  
See application file for complete search history.

(56)

**References Cited**

**U.S. PATENT DOCUMENTS**

|              |      |         |                    |
|--------------|------|---------|--------------------|
| 4,045,306    | A    | 8/1977  | Senge et al.       |
| 4,169,772    | A    | 10/1979 | Lowery et al.      |
| 4,374,709    | A *  | 2/1983  | Combs .....        |
| 4,397,717    | A    | 8/1983  | Acimovic et al.    |
| 4,730,022    | A    | 3/1988  | Willis             |
| 5,607,570    | A *  | 3/1997  | Rohbani .....      |
| 5,750,018    | A *  | 5/1998  | Brasch .....       |
| 7,128,822    | B2   | 10/2006 | Wang et al.        |
| 7,374,652    | B2   | 5/2008  | Hayashi et al.     |
| 2003/0102226 | A1 * | 6/2003  | Gabe et al. .....  |
| 2009/0075102 | A1 * | 3/2009  | Brese et al. ..... |

**OTHER PUBLICATIONS**

Joi et al.; "Additives for Bottom-up Copper Plating from an Alkaline Complexed Electrolyte"; Journal of The Electrochemical Society; 160 (12) 2013; pp. D3001-D3003.

\* cited by examiner

*Primary Examiner* — Edna Wong

(74) *Attorney, Agent, or Firm* — S. Matthew Cairns

**ABSTRACT**

Copper plating baths containing a leveling agent that is a reaction product of one or more of certain cyclodiazia-compounds with one or more epoxide-containing compounds that deposit copper on the surface of a conductive layer are provided. Such plating baths deposit a copper layer that is substantially planar on a substrate surface across a range of electrolyte concentrations. Methods of depositing copper layers using such copper plating baths are also disclosed.

**11 Claims, No Drawings**

**1**  
**PLATING BATH AND METHOD**

The present invention relates generally to the field of electrolytic metal plating. In particular, the present invention relates to the field of electrolytic copper plating.

Methods for electroplating articles with metal coatings generally involve passing a current between two electrodes in a plating solution where one of the electrodes is the article to be plated. A typical acid copper plating solution comprises dissolved copper (usually copper sulfate), an acid electrolyte such as sulfuric acid in an amount sufficient to impart conductivity to the bath, and proprietary additives to improve the uniformity of the plating and the quality of the metal deposit. Such additives include accelerators, levelers, and suppressors, among others.

Electrolytic copper plating solutions are used in a variety of industrial applications, such as decorative and anticorrosion coatings, as well as in the electronics industry, particularly for the fabrication of printed circuit boards and semiconductors. For circuit board fabrication, copper is electroplated over selected portions of the surface of a printed circuit board, into blind vias and onto the walls of through-holes passing between the surfaces of the circuit board base material. The walls of a through-hole are first made conductive, such as by electroless metal deposition, before copper is electroplated onto the walls of the through-hole. Plated through-holes provide a conductive pathway from one board surface to the other. For semiconductor fabrication, copper is electroplated over a surface of a wafer containing a variety of features such as vias, trenches or a combination thereof. The vias and trenches are metallized to provide conductivity between various layers of the semiconductor device.

It is well known in certain areas of plating, such as in electroplating of printed circuit boards ("PCBs"), that the use of accelerators and/or levelers in the electroplating bath can be crucial in achieving a uniform metal deposit on a substrate surface. Plating a substrate having irregular topography can pose particular difficulties. During electroplating, a voltage drop variation typically will exist along an irregular surface which can result in an uneven metal deposit. As a result, a thicker metal deposit, termed overplating, is observed over such surface irregularities. Consequently, a metal layer of substantially uniform thickness is frequently a challenging step in the manufacture of electronic devices. Leveling agents are often used in copper plating baths to provide substantially uniform, or level, copper layers in electronic devices.

The trend of portability combined with increased functionality of electronic devices has driven the miniaturization of PCBs. Approaches for high density interconnects have been developed, such as sequential build up technologies, which utilize blind vias. One of the objectives in processes that use blind vias is maximizing via filling while minimizing thickness variation in the copper deposit across the substrate surface. This is particularly challenging when the PCB contains both through holes and blind vias.

Generally, leveling agents used in copper plating baths provide better leveling of the deposit across the substrate surface but tend to worsen the throwing power of the electroplating bath. Throwing power is defined as the ratio of the hole center copper deposit thickness to its thickness at the surface. Newer PCBs are being manufactured that contain both through-holes and blind vias. Current bath additives, in particular current leveling agents, do not provide level copper deposits on the substrate surface and fill through-holes and/or fill blind vias effectively. There remains a need in the art for leveling agents for use in copper electroplating baths used in the manufacture of PCBs that provide level copper deposits

**2**

while not significantly affecting the throwing power of the bath, that is, the bath effectively fills blind vias and through-holes.

U.S. Pat. No. 5,607,570 (Rohbani) discloses a cyanide-free, alkaline (pH 9-14) copper strike plating bath for depositing copper on zinc which may include a reaction product of epichlorohydrin with a various nitrogen-containing compounds, including nitrogen-containing heterocycles such as imidazole, pyrazole, triazole, tetrazole, pyridazine and the like. The key to this patent is the use of these reaction products to provide a cyanide-free strike bath that is to be able to deposit copper on zinc without the unwanted contamination from iron which normally occurs during the electroplating of copper on zinc. Such iron contamination leads to iron being deposited during plating which forms a complex with the copper being deposited, and this complex weakens the adhesion between the copper and the zinc. Although not specifically stated in the patent, the reaction products are presumably present in the copper strike baths to prevent interference from iron contamination. These reaction products are not disclosed to be leveling agents, particularly for use in acid copper electroplating baths.

The present invention provides a copper electroplating bath comprising: a source of copper ions, an electrolyte, and a leveling agent, wherein the leveling agent is a reaction product of one or more cyclodiazia-compounds with one or more epoxide-containing compounds; wherein at least one cyclodiazia-compound has the formula (I)



wherein E=C(O) or CR<sup>3</sup>R<sup>4</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>2</sup> and R<sup>3</sup>, R<sup>3</sup> and R<sup>8</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring. The present invention further provides a method of depositing copper on a substrate including: contacting a substrate to be plated with copper into a copper electroplating bath comprising: a source of copper ions, an electrolyte, and a leveling agent, wherein the leveling agent is a reaction product of one or more cyclodiazia-compounds with one or more epoxide-containing compounds; wherein at least one cyclodiazia-compound has the formula (I)



wherein E=C(O) or CR<sup>3</sup>R<sup>4</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and

(C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>2</sup> and R<sup>3</sup>, R<sup>3</sup> and R<sup>5</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring; and applying a current density for a period of time sufficient to deposit a copper layer on the substrate.

Also provided by the present invention is a composition comprising a reaction product of one or more cyclodiazocompounds with one or more epoxide-containing compounds; wherein at least one cyclodiazocompound has the formula (I)



(I)

wherein E=C(O) or CR<sup>3</sup>R<sup>4</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>2</sup> and R<sup>3</sup>, R<sup>3</sup> and R<sup>5</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring; and wherein at least one epoxide-containing compound of the formulae



where Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>)alkenyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>11</sup>=((CR<sup>13</sup>R<sup>14</sup>)<sub>n</sub>O)<sub>n</sub>, (aryl-O)<sub>p</sub>, CR<sup>13</sup>R<sup>14</sup>-Z-CR<sup>13</sup>R<sup>14</sup>O or OZ<sup>1</sup>O; R<sup>12</sup>=(CH<sub>2</sub>)<sub>j</sub>; Al is (C<sub>5</sub>-C<sub>12</sub>)cycloalkyl or a 5- to 6-membered cyclicsulfone ring; Z=a 5- or 6-membered ring; Z<sup>1</sup> is R<sup>15</sup>OArOR<sup>15</sup>, (R<sup>16</sup>O)<sub>a</sub>Ar(O<sup>16</sup>)<sub>a</sub>, or (R<sup>16</sup>O)<sub>a</sub>Cy(O<sup>16</sup>)<sub>a</sub>; Z<sup>2</sup>=SO<sub>2</sub> or



Cy=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleneoxy; each a=1-

10; m=1-6; n=1-20; p=1-6; q=1-6; r=0-4; t=1-4; v=0-3; and y=0-6; wherein Y<sup>1</sup> and Y<sup>2</sup> may be taken together to form a (C<sub>8</sub>-C<sub>12</sub>)cyclic compound. Such reaction products are particularly useful as leveling agents for copper plating baths.

5 It has been surprisingly found that the present invention provides copper layers having a substantially level surface across a PCB substrate, even on substrates having very small features and on substrates having a variety of feature sizes. The copper layers deposited according to the present method have significantly reduced defects, such as nodules, as compared to copper deposits from electroplating baths using conventional leveling agents. Further, the present invention effectively deposits copper in through-holes and blind via holes, that is, the present copper plating baths have good 10 throwing power.

15 As used throughout this specification, the following abbreviations shall have the following meanings, unless the context clearly indicates otherwise: A=amperes; A/dm<sup>2</sup>=amperes per square decimeter; ° C.=degrees Centigrade; g=gram; 20 mg=milligram; L=liter; L/m=liters per minute; ppm=parts per million; µm=micron=micrometer; mm=millimeters; cm=centimeters; DI=deionized; mmol=millimoles; and mL=milliliter. All amounts are percent by weight and all ratios are molar ratios, unless otherwise noted. All numerical 25 ranges are inclusive and combinable in any order, except where it is clear that such numerical ranges are constrained to add up to 100%.

30 As used throughout the specification, “feature” refers to the geometries on a substrate. “Apertures” refer to recessed features including through-holes and blind vias. As used throughout this specification, the term “plating” refers to metal electroplating. “Deposition” and “plating” are used interchangeably throughout this specification. “Halide” refers to fluoride, chloride, bromide and iodide. Likewise, 35 “halo” refers to fluoro, chloro, bromo and iodo. The term “alkyl” includes linear, branched and cyclic alkyl. “Accelerator” refers to an organic additive that increases the plating rate of the electroplating bath. A “suppressor” refers to an organic additive that suppresses the plating rate of a metal during 40 electroplating. “Leveler” refers to an organic compound that is capable of providing a substantially level (or planar) metal layer. The terms “leveler” and “leveling agent” are used interchangeably throughout this specification. The terms “printed 45 circuit boards” and “printed wiring boards” are used interchangeably throughout this specification. The articles “a” and “an” refer to the singular and the plural.

The plating bath and method of the present invention are useful in providing a substantially level plated copper layer on a substrate, such as a printed circuit board. Also, the 50 present invention is useful in filling apertures in a substrate with copper. Such filled apertures are substantially free of voids. Also, the copper deposits from the present invention are substantially free of nodules, that is, they contain ≤15 nodules/95 cm<sup>2</sup>, and preferably ≤10 nodules/95 cm<sup>2</sup>.

55 Any substrate upon which copper can be electroplated is useful in the present invention. Such substrates include, but are not limited to, electronic devices such as printed wiring boards, integrated circuits, semiconductor packages, lead frames and interconnects. It is preferred that the substrate is a 60 PCB or an integrated circuit. In one embodiment, the integrated circuit substrate is a wafer used in a dual damascene manufacturing process. Such substrates typically contain a number of features, particularly apertures, having a variety of sizes. Through-holes in a PCB may have a variety of diameters, such as from 50 µm to 150 µm in diameter. Such through-holes may vary in depth, such as from 35 µm to 100 µm. PCBs may contain blind vias having a wide variety of 65

sizes, such as up to 200  $\mu\text{m}$ , or greater. The present invention is particularly suitable for filling apertures, of varying aspect ratios, such as low aspect ratio vias and high aspect ratio apertures. By "low aspect ratio" is meant an aspect ratio of from 0.1:1 to 4:1. The term "high aspect ratio" refers to aspect ratios of greater than 4:1, such as 10:1 or 20:1.

The copper plating baths of the present invention contain a source of copper ions, an electrolyte, and a leveling agent, wherein the leveling agent is a reaction product of one or more cyclodiazia-compounds with one or more epoxide-containing compounds; wherein at least one cyclodiazia-compound has the formula (I)



(I)

wherein E=C(O) or CR<sup>3</sup>R<sup>4</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>2</sup> and R<sup>3</sup>, R<sup>3</sup> and R<sup>5</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring. The copper plating baths also typically contain a source of halide ions, an accelerator and a suppressor.

Any copper ion source that is at least partially soluble in the electroplating bath is suitable. Preferably, the copper ion source is soluble in the plating bath. Suitable copper ion sources are copper salts and include without limitation: copper sulfate; copper halides such as copper chloride; copper acetate; copper nitrate; copper fluoroborate; copper alkylsulfonates; copper arylsulfonates; copper sulfamate; and copper gluconate. Exemplary copper alkylsulfonates include copper (C<sub>1</sub>-C<sub>6</sub>)alkylsulfonate and more preferably copper (C<sub>1</sub>-C<sub>3</sub>) alkylsulfonate. Preferred copper alkylsulfonates are copper methanesulfonate, copper ethanesulfonate and copper propanesulfonate. Exemplary copper arylsulfonates include, without limitation, copper phenyl sulfonate, copper phenol sulfonate and copper p-toluenesulfonate. Copper sulfate pentahydrate and copper methanesulfonic acid are preferred. Mixtures of copper ion sources may be used. It will be appreciated by those skilled in the art that one or more salts of metal ions other than copper ions may be advantageously added to the present electroplating baths. The addition of such other metal ion sources is useful in the deposition of copper alloys. Such copper salts are generally commercially available and may be used without further purification.

The copper salts may be used in the present plating baths in any amount that provides sufficient copper ion concentration for electroplating copper on a substrate. Typically, the copper salt is present in an amount sufficient to provide an amount of copper metal of 10 to 180 g/L of plating solution. Alloys, such as copper-tin, for example, copper having up to 2% by weight tin, may be advantageously plated according to the present invention. Other suitable copper alloys include, but are not limited to copper-silver, tin-copper-silver, and tin-copper-bismuth. The amount of each of the metal salts in such mix-

tures depends upon the particular alloy to be plated and is well known to those skilled in the art.

The electrolyte useful in the present invention may be alkaline or acidic. Suitable acidic electrolytes include, but are not limited to, sulfuric acid, acetic acid, fluoroboric acid, alkanesulfonic acids such as methanesulfonic acid, ethanesulfonic acid, propanesulfonic acid and trifluoromethane sulfonic acid, arylsulfonic acids such as phenyl sulfonic acid, phenol sulfonic acid and toluene sulfonic acid, sulfamic acid, hydrochloric acid, and phosphoric acid. Mixtures of acids may be advantageously used in the present metal plating baths. Preferred acids include sulfuric acid, methanesulfonic acid, ethanesulfonic acid, propanesulfonic acid, and mixtures thereof. The acids are typically present in an amount in the range of from 1 to 300 g/L, preferably from 5 to 250 g/L, and more preferably from 10 to 225 g/L. Electrolytes are generally commercially available from a variety of sources and may be used without further purification.

Such electrolytes may optionally contain a source of halide ions. Chloride ions are the preferred halide ions. Exemplary chloride ion sources include copper chloride and hydrochloric acid. A wide range of halide ion concentrations may be used in the present invention. Typically, the halide ion concentration is in the range of from 0 to 100 ppm based on the plating bath, and preferably from 10 to 100 ppm. A more preferable amount of halide ion is from 20 to 75 ppm. Such halide ion sources are generally commercially available and may be used without further purification.

The present plating baths typically contain an accelerator. Any accelerators (also referred to as brightening agents) are suitable for use in the present invention and are well-known to those skilled in the art. Typical accelerators contain one or more sulfur atoms and have a molecular weight of 1000 or less. Accelerator compounds that have sulfide and/or sulfonic acid groups are generally preferred, particularly compounds that include a group of the formula R'-S-R-SO<sub>3</sub>X, where R is optionally substituted alkyl, optionally substituted heteroalkyl, optionally substituted aryl, or optionally substituted heterocyclic; X is a counter ion such as sodium or potassium; and R' is hydrogen or a chemical bond. Typically, the alkyl groups are (C<sub>1</sub>-C<sub>16</sub>)alkyl and preferably (C<sub>3</sub>-C<sub>12</sub>)alkyl. Heteroalkyl groups typically have one or more heteroatoms, such as nitrogen, sulfur or oxygen, in the alkyl chain. Suitable aryl groups include, but are not limited to, phenyl, benzyl, biphenyl and naphthyl. Suitable heterocyclic groups typically contain from 1 to 3 heteroatoms, such as nitrogen, sulfur or oxygen, and 1 to 3 separate or fused ring systems. Such heterocyclic groups may be aromatic or non-aromatic. Preferred accelerators include: N,N-dimethyl-dithiocarbamic acid-(3-sulfopropyl)ester; 3-mercaptopropropylsulfonic acid-(3-sulfopropyl)ester; 3-mercaptopropropylsulfonic acid sodium salt; carbonic acid-dithio-o-ethylester-s-ester with 3-mercaptopropane sulfonic acid potassium salt; bis-sulfopropyl disulfide; 3-(benzothiazolyl-s-thio)propyl sulfonic acid sodium salt; pyridinium propyl sulfobetaine; 1-sodium-3-mercaptopropane-1-sulfonate; N,N-dimethyl-dithiocarbamic acid-(3-sulfoethyl)ester; 3-mercaptopropanylsulfonic acid-(3-sulfoethyl)ester; 3-mercaptopropanylsulfonic acid sodium salt; carbonic acid-dithio-o-ethylester-s-ester with 3-mercaptopropane sulfonic acid potassium salt; bis-sulfopropyl disulfide; 3-(benzothiazolyl-s-thio)propyl sulfonic acid sodium salt; pyridinium ethyl sulfobetaine; and 1-sodium-3-mercaptopropane-1-sulfonate.

Such accelerators may be used in a variety of amounts. In general, accelerators are used in an amount of at least 0.01 mg/L, based on the bath, preferably at least 0.5 mg/L, and more preferably at least 1 mg/L. For example, the accelerators

are present in an amount of from 0.1 mg/L to 200 mg/L. The particular amount of accelerator will depend upon the specific application, such as high aspect ratio, through-hole filling, and via filling applications. Preferable amounts of accelerator are at least 0.5 mg/L, and more preferably at least 1 mg/L. A preferable range of such accelerator concentrations is from 0.1 to 10 mg/L (ppm).

Any compound capable of suppressing the copper plating rate may be used as a suppressor in the present electroplating baths. Suitable suppressors include, but are not limited to, polymeric materials, particularly those having heteroatom substitution, and more particularly oxygen substitution. Exemplary suppressors are high molecular weight polyethers, such as those of the formula  $R-O-(CX_2CY_2X'Y'O)_nR'$  where  $R$  and  $R'$  are independently chosen from H,  $(C_2-C_{20})$ alkyl group and  $(C_6-C_{10})$ aryl group; each of  $X$ ,  $Y$ ,  $X'$  and  $Y'$  is independently selected from hydrogen, alkyl such as methyl, ethyl or propyl, aryl such as phenyl, or aralkyl such as benzyl; and  $n$  is an integer from 5 to 100,000. Typically, one or more of  $X$ ,  $Y$ ,  $X'$  and  $Y'$  is hydrogen. Preferred suppressors include commercially available polypropylene glycol copolymers and polyethylene glycol copolymers, including ethylene oxide-propylene oxide ("EO/PO") copolymers and butyl alcohol-ethylene oxide-propylene oxide copolymers. Suitable butyl alcohol-ethylene oxide-propylene oxide copolymers are those having a weight average molecular weight of 500 to 10,000, and preferably 1000 to 10,000. When such suppressors are used, they are typically present in an amount in the range of from 1 to 10,000 ppm based on the weight of the bath, and preferably from 5 to 10,000 ppm.

The reaction products of the present invention contain at least one cyclodiaza-compound of the formula (I)



(I) 35

wherein  $E=C(O)$  or  $CR^3R^4$ ;  $G=CR^5R^6$  or a chemical bond;  $R^1$  and  $R^2$  are independently chosen from H,  $(C_1-C_6)$ alkyl and  $(C_6-C_{10})$ aryl;  $R^3$  to  $R^{10}$  are independently chosen from H,  $(C_1-C_6)$ alkyl,  $(C_6-C_{10})$ aryl and hydroxyl; each of  $R^1$  and  $R^2$ ,  $R^2$  and  $R^3$ ,  $R^3$  and  $R^5$ ,  $R^5$  and  $R^7$ ,  $R^7$  and  $R^9$ , and  $R^9$  and  $R^1$  may be taken together to form a chemical bond; and any of  $R^1$  to  $R^{10}$  on adjacent ring atoms may be taken together along with the atoms to which they are attached to form a 5- or 6-membered saturated or unsaturated ring. Any of the  $(C_1-C_6)$ alkyl and  $(C_6-C_{10})$ aryl groups of any of  $R^1$  to  $R^{10}$  may optionally be substituted. As used herein, the term "substituted" refers to the replacement of one or more hydrogen atoms with one or more of halide, hydroxy or  $(C_1-C_3)$ alkoxy. " $(C_6-C_{10})$ Aryl," as used herein, includes, but is not limited to, phenyl, naphthyl, benzyl, phenethyl, and  $(C_1-C_4)$ alkylphenyl. It is preferred that  $G$  is a chemical bond. Preferably,  $R^1$  and  $R^2$  are independently chosen from H,  $(C_1-C_3)$ alkyl and  $(C_6-C_8)$ aryl. More preferably,  $R^1$  and  $R^2$  are independently chosen from H, methyl, ethyl, phenyl, methylphenyl, ethylphenyl, benzyl and phenethyl. It is preferred that  $R^3$  to  $R^{10}$  are independently chosen from H,  $(C_1-C_3)$ alkyl,  $(C_6-C_8)$ aryl and hydroxyl, and more preferably from H, methyl, ethyl, phenyl, methylphenyl, ethylphenyl, benzyl, phenethyl and hydroxyl.

Preferred cyclodiaza-compounds when  $G$  is a chemical bond include compounds of formulae (IIa) and (IIb)



(IIa)



(IIb)

wherein  $R^1$  and  $R^2$  are independently chosen from H,  $(C_1-C_6)$ alkyl and  $(C_6-C_{10})$ aryl;  $R^4$  and  $R^7$  to  $R^{10}$  are independently chosen from H,  $(C_1-C_6)$ alkyl,  $(C_6-C_{10})$ aryl and hydroxyl;  $R^7$  and  $R^9$  may be taken together to form a chemical bond; and any of  $R^1$ ,  $R^4$  and  $R^7$  to  $R^{10}$  on adjacent ring atoms may be taken together along with the atoms to which they are attached to form a 5- or 6-membered saturated or unsaturated ring. It is more preferred that  $R^1$  and  $R^2$  are independently chosen from H, methyl, phenyl, benzyl and methylphenyl, even more preferably from H, methyl and phenyl, and most preferably from H and phenyl. In formula IIa,  $R^1$  is preferably H. In formula IIb, at least one of  $R^1$  and  $R^2$  is preferably H. Preferably,  $R^4$  and  $R^7$  to  $R^{10}$  are independently chosen from H,  $(C_1-C_3)$ alkyl,  $(C_6-C_8)$ aryl and hydroxyl, and more preferably from H, methyl, phenyl, hydroxyphenyl, benzyl, methylphenyl, and methoxyphenyl, and most preferably from H, methyl, phenyl, and hydroxyphenyl. It is preferred that when any of  $R^1$ ,  $R^4$  and  $R^7$  to  $R^{10}$  on adjacent ring atoms be taken together along with the atoms to which they are attached to form a ring, they form a 6-membered ring. Particularly preferred compounds of formulae (IIa) and (IIb) are pyrazole, 3-methylpyrazole, 4-methylpyrazole, 3,4-dimethylpyrazole, 3,5-dimethylpyrazole, 3-phenylpyrazole, 3,5-diphenylpyrazole, 3-(2-hydroxyphenyl)pyrazole, indazole, 4,5,6,7-tetrahydroindazoles, 3-methyl-3-pyrazolin-5-one, 4-methyl-2-pyrazolin-5-one, 1-phenyl-3-pyrazolidinone, and 1-phenyl-4,4-dimethyl-3-pyrazolidinone.

Preferred cyclodiaza-compounds when  $G=CR^5R^6$  include compounds of formulae (IIIa) and (IIIb)



(IIIa)



(IIIb)

9

wherein  $R^1$  and  $R^2$  are independently chosen from H, ( $C_1$ - $C_6$ )alkyl and ( $C_6$ - $C_{10}$ )aryl;  $R^4$  and  $R^5$  to  $R^{10}$  are independently chosen from H, ( $C_1$ - $C_6$ )alkyl, ( $C_6$ - $C_{10}$ )aryl and hydroxyl; each of  $R^1$  and  $R^2$ ,  $R^5$  and  $R^7$ ,  $R^7$  and  $R^9$ , and  $R^9$  and  $R^1$  may be taken together to form a chemical bond; and any of  $R^1$  and  $R^5$  to  $R^{10}$  on adjacent ring atoms may be taken together along with the atoms to which they are attached to form a 5- or 6-membered saturated or unsaturated ring. It is more preferred that  $R^1$  and  $R^2$  are independently chosen from H, methyl, phenyl, benzyl and methylphenyl, even more preferably from H, methyl and phenyl, and most preferably H. Preferably,  $R^1$  and  $R^9$  are taken together to form a chemical bond, and even more preferably each of  $R^1$  and  $R^9$ , and  $R^5$  and  $R^7$ , are taken together to form chemical bonds. Preferably,  $R^4$  and  $R^5$  to  $R^{10}$  are independently chosen from H, ( $C_1$ - $C_3$ )alkyl, ( $C_6$ - $C_8$ )aryl and hydroxyl, and more preferably from H, methyl, phenyl, hydroxyphenyl, benzyl, methylphenyl, hydroxyphenyl, chlorophenyl, and methoxyphenyl, and most preferably from H, methyl, phenyl, hydroxyphenyl, and chlorophenyl. It is preferred that when any of  $R^1$ ,  $R^4$  and  $R^5$  to  $R^{10}$  on adjacent ring atoms be taken together along with the atoms to which they are attached to form a ring, they form a 6-membered ring. Particularly preferred compounds of formulae (IIIa) and (IIIb) are pyridazine, 3-methylpyridazine, 4-methylpyridazine, 3,6-dihydroxypyridazine, 3,6-dihydroxy-4-methyl-pyridazine, phthalazine, 6-phenyl-3(2H)-pyridazinone, 6-(2-hydroxyphenyl)-3(2H)-pyridazinone, 4,5-dihydro-6-phenyl-3(2H)-pyridazinone, 1(2H)-phthalazinone, 4-phenylphthalazin-1(2H)-one, 4-(4-methylphenyl)phthalazin-1(2H)-one, and 4-(4-chlorophenyl)phthalazin-1(2H)-one.

The cyclodiazia-compounds useful in the present invention are generally commercially available from a variety of sources, such as Sigma-Aldrich (St. Louis, Mo.) or may be prepared from literature methods. These compounds may be used as-is, or may be purified before being reacted with the one or more epoxy-containing compounds.

Any suitable epoxide-containing compound may be used to make the reaction products of the present invention. Such epoxide-containing compounds may contain 1 or more epoxide groups, and typically contain 1, 2 or 3 epoxide groups, and preferably contain 1 or 2 epoxide groups. Suitable epoxide-containing compounds useful in the present invention are those of the formulae E-I, E-II, or E-III.



where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>)alkenyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>11</sup>=((CR<sup>13</sup>R<sup>14</sup>)<sub>n</sub>O)...

10

(aryl-O)<sub>p</sub>, CR<sup>13</sup>R<sup>14</sup>-Z-CR<sup>13</sup>R<sup>14</sup>O or OZ<sup>1</sup><sub>1</sub>O; R<sup>12</sup>=  
(CH<sub>2</sub>)<sub>y</sub>; Al is a (C<sub>5</sub>-C<sub>12</sub>)cycloalkyl ring or a 5- to 6-membered  
cyclicsulfone ring; Z=a 5- or 6-membered ring; Z<sup>1</sup> is  
R<sup>15</sup>OArOR<sup>15</sup>, (R<sup>16</sup>O)<sub>a</sub>Ar(O<sup>16</sup>)<sub>a</sub>, or (R<sup>16</sup>O)<sub>a</sub>Cy(O<sup>16</sup>)<sub>a</sub>;  
Z<sup>2</sup>=SO<sub>2</sub> or



Cy=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleneoxy; each a=1-10; m=1-6; n=1-20; p=1-6; q=1-6; r=0-4; t=1-4; v=0-3; and y=0-6; wherein Y<sup>1</sup> and Y<sup>2</sup> may be taken together to form a (C<sub>8</sub>-C<sub>12</sub>)cyclic compound. Preferably Y=H. More preferably X<sup>1</sup>=H. It is preferred that X=CH<sub>2</sub>X<sup>2</sup>. It is further preferred that X<sup>2</sup>=halogen or O(C<sub>1</sub>-C<sub>3</sub>)fluoroalkyl. Even more preferred are compounds of formula E-I where Y=X<sup>1</sup>=H, X=CH<sub>2</sub>X<sup>2</sup> and X<sup>2</sup>=Cl or Br, and more preferably, X<sup>2</sup>=Cl. Y<sup>1</sup> and Y<sup>2</sup> are preferably independently chosen from H and (C<sub>1</sub>-C<sub>2</sub>)alkyl. When Y<sup>1</sup> and Y<sup>2</sup> are not joined to form a cyclic compound, it is preferred that Y<sup>1</sup> and Y<sup>2</sup> are both H. When Y<sup>1</sup> and Y<sup>2</sup> are joined to form a cyclic compound, it is preferred that A is R<sup>12</sup> or a chemical bond and that a (C<sub>8</sub>-C<sub>10</sub>) carbocyclic ring is formed. It is preferred that m=2-4. Preferably, n=1-10. It is further preferred that m=2-4 when n=1-10. Phenyl-O is the preferred aryl-O group for R<sup>11</sup>. It is preferred that p=1-4, more preferably 1-3, and still more preferably 1-2. Z is preferably a 5- or 6-membered carbocyclic ring and, more preferably, Z is a 6-membered carbocyclic ring. Preferably, Z<sup>2</sup> is



It is preferred that  $v=0-2$ . Preferably,  $y=0-4$ , and more preferably 1-4. When  $A=R^{12}$  and  $y=0$ , then  $A$  is a chemical bond. Preferably,  $m=1-6$ , and more preferably 1-4. It is preferred that  $q=1-4$ , more preferably 1-3, and still more preferably 1-2. 45 Preferably,  $r=0$  and  $q=1$ , and more preferably  $Y^1$  and  $Y^2=H$ ,  $r=0$  and  $q=1$ . Preferably,  $Z^1=R^{15}OArOR^{15}$  or  $(R^{16}O)_aAr(OR^{16})_a$ . Each  $R^{15}$  is preferably  $(C_1-C_6)alkyl$  and more preferably  $(C_1-C_4)alkyl$ . Each  $R^{16}$  is preferably  $(C_2-C_4)alkyleoxy$ . It is preferred that  $t=1-2$ . Preferably,  $a=1-8$ , more 50 preferably 1-6 and still more preferably 1-4. When  $Z^2$  is



it is preferred that A1 is a 6- to 10-membered carbocyclic ring, and more preferably a 6- to 8-membered carbocyclic ring.

Exemplary epoxide-containing compounds of formula E-1 include, without limitation, epihalohydrin, 1,2-epoxy-5-hexene, 2-methyl-2-vinyloxirane, and glycidyl 1,1,2,2-tetrafluoroethyl ether. Preferably, the epoxide-containing compound is epichlorohydrin or epibromohydrin, and more preferably epichlorohydrin.

Suitable compounds of formula E-II where  $R^{11} = ((CR^{13}R^{14})_mO)_n$  are those of the formula:

11



(E-IIa)

5

where  $Y^1$ ,  $Y^2$ ,  $R^{13}$ ,  $R^{14}$ ,  $n$  and  $m$  are as defined above. Preferably,  $Y^1$  and  $Y^2$  are both H. When  $m=2$ , it is preferred that each  $R^{13}$  is H,  $R^{14}$  is chosen from H and  $CH_3$ , and  $n=1-10$ . When  $m=3$ , it is preferred that at least one  $R^{14}$  is chosen from  $CH_3$  and OH, and  $n=1$ . When  $m=4$ , it is preferred that both  $R^{13}$  and  $R^{14}$  are H, and  $n=1$ . Exemplary compounds of formula E-IIa include, but are not limited to: 1,4-butanediol diglycidyl ether, ethylene glycol diglycidyl ether, di(ethylene glycol) diglycidyl ether, poly(ethylene glycol)diglycidyl ether compounds, glycerol diglycidyl ether, neopentyl glycol diglycidyl ether, propylene glycol diglycidyl ether, di(propylene glycol)diglycidyl ether, and poly(propylene glycol)diglycidyl ether compounds. Poly(ethylene glycol)diglycidyl ether compounds of formula E-IIa are those compounds where each of  $R^{13}$  and  $R^{14}=H$ ,  $m=2$ , and  $n=3-20$ , and preferably  $n=3-15$ , more preferably  $n=3-12$ , and still more preferably  $n=3-10$ . Exemplary poly(ethylene glycol)diglycidyl ether compounds include tri(ethylene glycol)diglycidyl ether, tetra(ethylene glycol)diglycidyl ether, penta(ethylene glycol) diglycidyl ether, hexa(ethylene glycol)diglycidyl ether, nona(ethylene glycol)diglycidyl ether, deca(ethylene glycol)diglycidyl ether, and dodeca(ethylene glycol) diglycidyl ether. Poly(propylene glycol)diglycidyl ether compounds of formula E-IIa are those compounds where each of  $R^{13}=H$  and one of  $R^{14}=CH_3$ ,  $m=2$ , and  $n=3-20$ , and preferably  $n=3-15$ , more preferably  $n=3-12$ , and still more preferably  $n=3-10$ . Exemplary poly(propylene glycol)diglycidyl ether compounds include tri(propylene glycol)diglycidyl ether, tetra(propylene glycol)diglycidyl ether, penta(propylene glycol) diglycidyl ether, hexa(propylene glycol)diglycidyl ether, nona(propylene glycol)diglycidyl ether, deca(propylene glycol)diglycidyl ether, and dodeca(propylene glycol)diglycidyl ether. Suitable poly(ethylene glycol)diglycidyl ether compounds and poly(propylene glycol)diglycidyl ether compounds are those having a number average molecular weight of from 200 to 10000, and preferably from 350 to 8000.

Suitable compounds of formula E-II where  $R^{11}=(\text{aryl-O})_p$  are those having the formulae E-IIb, E-IIc and E-IId:

12

-continued

(E-IId)



10

15

where  $Y^1$ ,  $Y^2$  and  $p$  are as defined above, and each  $R^{17}$  represents  $(C_1-C_4)$ alkyl or  $(C_1-C_4)$ alkoxy, and  $r=0-4$ . Preferably,  $r=0$  and  $p=1$ , and more preferably  $Y^1$  and  $Y^2=H$ ,  $r=0$  and  $p=1$ . Exemplary compounds include, without limitation, tris(4-hydroxyphenyl)methane triglycidyl ether, bis(4-hydroxyphenyl)methane diglycidyl ether, and resorcinol diglycidyl ether.

In compounds of formula E-II where  $R^{11}=CR^{13}R^{14}-Z-CR^{13}R^{14}O$ ,  $Z$  represents a 5- or 6-membered ring. In such ring structures, the  $CR^{13}R^{14}$  groups may be attached at any position, such as at adjacent atoms of the ring or at any other atoms of the ring. Particularly suitable compounds of formula E-II where  $R^{11}=CR^{13}R^{14}-Z-CR^{13}R^{14}O$  are those having the formula



35

40

where  $Y^1$ ,  $Y^2$ ,  $R^{13}$  and  $R^{14}$  are as defined above, and  $q=0$  or 1. When  $q=0$ , the ring structure is a 5-membered carbocyclic ring and when  $q=1$ , the ring structure is a 6-membered carbocyclic ring. Preferably,  $Y^1$  and  $Y^2=H$ . More preferably,  $Y^1$  and  $Y^2=H$  and  $q=1$ . Preferred compounds of formula E-II where  $R^{11}=CR^{13}R^{14}-Z-CR^{13}R^{14}O$  are 1,2-cyclohexanediol diglycidyl ether and 1,4-cyclohexanediol diglycidyl ether.

When  $A=R^{12}$ , suitable compounds of formula E-II are those having the formula:



(E-IIb)  
(E-IIc)

(E-IIe)

where  $Y^1$ ,  $Y^2$  and  $y$  are as defined above. It is preferred that  $y=0-4$ , more preferably  $y=1-4$ , and  $y=2-4$ . Exemplary compounds of formula E-IIe include, without limitation: 1,2,5,6-diepoxyhexane; 1,2,7,8-diepoxyoctane; and 1,2,9,10-diepoxydecane.



65



In compounds of formula II where  $A=OZ^{12}O$ , preferred compounds are those of the formula



wherein Y<sup>1</sup> and Y<sup>2</sup> are as defined above.

Suitable epoxy-containing compounds of formula E-III may be monocyclic, spirocyclic, fused and/or bicyclic rings. Preferred epoxide-containing compounds of formula E-III include 1,2,5,6-diepoxy-cyclooctane, 1,2,6,7-diepoxy-cyclodecane, dicyclopentadiene dioxide, 3,4-epoxytetrahydrothiophene-1,1-dioxide, cyclopentene oxide, cyclohexene oxide, and vinylcyclohexene dioxide.

The epoxide-containing compounds useful in the present invention can be obtained from a variety of commercial sources, such as Sigma-Aldrich, or can be prepared using a variety of literature methods known in the art.

The reaction products of the present invention can be prepared by reacting one or more cyclodiaza-compounds described above with one or more epoxide-containing compounds described above. Typically, a desired amount of the cyclodiaza-compounds and epoxide-containing compounds are added into the reaction flask, followed by addition of water. The resulting mixture is heated to approximately to 75-95° C. for 4 to 6 hours. After an additional 6-12 hours of stirring at room temperature, the resulting reaction product is diluted with water. The reaction product may be used as-is in aqueous solution, may be purified or may be isolated as desired.

In general, the present leveling agents have a number average molecular weight (Mn) of 500 to 10,000, although reaction products having other Mn values may be used. Such reaction products may have a weight average molecular weight (Mw) value in the range of 1000 to 50,000, although other Mw values may be used. The Mw values are determined using size exclusion chromatography and a PL Aquagel-OH 8 μm, 300×7.5 mm column from Varian, Inc. and polyethylene glycol calibration kit standards from Polymer Standards Service-USA, Inc. Typically, Mw is from 1000 to 20,000, preferably from 1000 to 15,000, and more preferably from Mw is 1500 to 5000.

Typically, the ratio of the cyclodiaza-compound to the epoxide-containing compound is from 0.1:10 to 10:0.1. Preferably, the ratio is from 0.5:5 to 5:0.5 and more preferably from 0.5:1 to 1:0.5. Other suitable ratios of cyclodiaza-compound to epoxide-containing compound may be used to prepare the present leveling agents.

It will be appreciated by those skilled in the art that a leveling agent of the present invention may also possess functionality capable of acting as a suppressor. Such compounds may be dual-functioning, i.e. they may function as leveling agents and as suppressors.

The amount of the leveling agent used in the metal electroplating baths will depend upon the particular leveling agents selected, the concentration of the metal ions in the electroplating bath, the particular electrolyte used, the concentration of the electrolyte and the current density applied. In general, the total amount of the leveling agent in the electroplating bath is from 0.01 ppm to 5000 ppm based on the total weight of the plating bath, although greater or lesser amounts may be used. Preferably, the total amount of the

(E-IIIf)

10 leveling agent is from 0.25 to 5000 ppm and more typically from 0.25 to 1000 ppm and still more preferably from 0.25 to 100 ppm.

15 The leveling agents of the present invention may possess any suitable molecular weight polydispersity. The present leveling agents work over a wide molecular weight polydispersity range.

20 The electroplating baths of the present invention are typically aqueous. Unless otherwise specified, all concentrations of components are in an aqueous system. Particularly suitable compositions useful as electroplating baths in the present invention include a soluble copper salt, an acid electrolyte, an accelerator, a suppressor, halide ion and a reaction product described above as a leveling agent. More preferably, suitable 25 compositions include 10 to 220 g/L of a soluble copper salts as copper metal, 5 to 250 g/L of acid electrolyte, 1 to 50 mg/L of an accelerator, 1 to 10,000 ppm of a suppressor, 10 to 100 ppm of a halide ion, and 0.25 to 5000 ppm of a reaction product described above as a leveling agent.

30 The electroplating baths of the present invention may be prepared by combining the components in any order. It is preferred that the inorganic components such as source of copper ions, water, electrolyte and optional halide ion source, are first added to the bath vessel followed by the organic 35 components such as leveling agent, accelerator, suppressor, and any other organic component.

35 The present electroplating baths may optionally contain a second leveling agent. Such second leveling agent may be another leveling agent of the present invention, or alternatively, 40 may be any conventional leveling agent. Suitable conventional leveling agents that can be used in combination with the present leveling agents include, without limitations, those disclosed in U.S. Pat. No. 6,610,192 (Step et al.), U.S. Pat. No. 7,128,822 (Wang et al.), U.S. Pat. No. 7,374,652 (Hayashi et al.), and U.S. Pat. No. 6,800,188 (Hagiwara et al.), and in U.S. patent application Ser. No. 12/661,301 (Niazimbetova et al.), filed on Mar. 15, 2010, now abandoned, Ser. No. 12/661,311 (Niazimbetova et al.), filed on Mar. 15, 2010, now U.S. Pat. No. 8,268,895, and 12/661,312 (Niazimbetova) filed on Mar. 15, 2010, now U.S. Pat. No. 8,268,157.

45 The plating baths of the present invention may be used at any suitable temperature, such as from 10 to 65° C. or higher. Preferably, the temperature of the plating baths is from 10 to 35° C. and more preferably from 15 to 30° C.

50 In general, the present copper electroplating baths are agitated during use. Any suitable agitation method may be used with the present invention and such methods are well-known in the art. Suitable agitation methods include, but are not limited to, air sparging, work piece agitation, and impingement.

55 Typically, a substrate is electroplated by contacting the substrate with the plating bath of the present invention. The substrate typically functions as the cathode. The plating bath contains an anode, which may be soluble or insoluble. Potential is typically applied to the cathode. Sufficient current density is applied and plating performed for a period of time 60 sufficient to deposit a copper layer having a desired thickness

## 15

on the substrate as well as fill blind vias and/or through holes. Suitable current densities, include, but are not limited to, the range of 0.05 to 10 A/dm<sup>2</sup>, although higher and lower current densities may be used. The specific current density depends in part upon the substrate to be plated and the leveling agent selected. Such current density choice is within the abilities of those skilled in the art.

The present invention is useful for depositing a copper layer on a variety of substrates, particularly those having variously sized apertures. Accordingly, the present invention provides a method of depositing a copper layer on a substrate including the steps of: contacting a substrate to be plated with copper with the copper plating bath described above; and then applying a current density for a period of time sufficient to deposit a copper layer on the substrate. For example, the present invention is particularly suitable for depositing copper on printed circuit boards with blind vias and through-holes.

Copper is deposited in apertures according to the present invention without substantially forming voids within the metal deposit. By the term "without substantially forming voids", it is meant that >95% of the plated apertures are void-free. It is preferred that the plated apertures are void-free. Copper is also deposited uniformly in through-holes and in high aspect ratio through-holes with improved throwing power, surface distribution and thermal reliability.

While the process of the present invention has been generally described with reference to printed circuit board manufacture, it will be appreciated that the present invention may be useful in any electrolytic process where an essentially level or planar copper deposit and filled apertures that are substantially free of voids are desired. Such processes include semiconductor packaging and interconnect manufacture.

An advantage of the present invention is that substantially level copper deposits are obtained on a PCB. By "substantially level" copper layer is meant that the step height, that is, the difference between areas of dense very small apertures and areas free of or substantially free of apertures, is less than 5  $\mu$ m, and preferably less than 1  $\mu$ m. Through-holes and/or blind vias in the PCB are substantially filled with substantially no void formation. A further advantage of the present invention is that a wide range of apertures and aperture sizes may be filled within a single substrate with substantially no suppressed local plating. Thus, the present invention is particularly suitable for filling blind vias and/or through-holes in a printed circuit board, where such blind vias and through-holes are substantially free of added defects. "Substantially free of added defects" refers to the leveling agent not increasing the number or size of defects, such as voids, in filled apertures as compared to control plating baths not containing

## 16

such leveling agent. A further advantage of the present invention is that a substantially planar copper layer may be deposited on a PCB having non-uniformly sized apertures. "Non-uniformly sized apertures" refer to apertures having a variety of sizes in the same PCB.

## EXAMPLE 1

In 100 mL round-bottom, three-neck flask equipped with a condenser and a thermometer, 100 mmol of pyrazole and 20 mL of DI water were added followed by addition of 63 mmol of 1,4-butanediol diglycidyl ether. The resulting mixture was heated for about 5 hours using an oil bath set to 110°C. and then left to stir at room temperature for additional 8 hours. An amber colored not-very viscous reaction product was transferred into a 200 mL volumetric flask, rinsed and adjusted with DI water to the 200 mL mark. The reaction product (Reaction Product 1) solution was used without further purification. Analysis of Reaction Product 1 by <sup>1</sup>H NMR (500 MHz, CH<sub>3</sub>OH-d6) showed the following peaks, confirming the structure:  $\delta$  ppm: 7.65-7.62 (m, 1H, H<sub>arom.</sub>); 7.49-7.48 (m, 1H, H<sub>arom.</sub>); 6.29-6.27 (m, 1H, H<sub>arom.</sub>); 4.32-3.30 (m, 8.82H (14H $\times$ 0.63 mole), 4 $\times$ CH<sub>2</sub>-O, 2 $\times$ CH-OH, 2 $\times$ CH<sub>2</sub>-N); 1.69-1.63 (m, 2.52H (4H $\times$ 0.63 mole), 2 $\times$ CH<sub>2</sub>).

## EXAMPLE 2

1,4-Butanediol diglycidyl ether (25.2 mmol) and 40 mmol of 4,5,6,7-tetrahydroindazole were added at room temperature to a round-bottom reaction flask. Next, 12 mL of DI water were added to the flask. The initially formed white colored suspension eventually disappeared as the reaction temperature increased and turned into a phase separated mixture. The reaction mixture was heated for 2 hours using an oil bath set to 95°C. After adding 2 mL of concentrated (or 4 ml of 50%) sulfuric acid into the reaction flask, the solution became transparent with a light-yellow color. The mixture was heated for an additional 3 hours and left stirring at room temperature for another 8 hours. The resulting light amber colored reaction product was transferred into a volumetric flask, rinsed and diluted with 0.5-1% sulfuric acid. The reaction product (Reaction Product 2) solution was used without further purification.

## EXAMPLE 3

The reaction products in Table 1 were prepared using the general procedures of Examples 1 or 2. The UV-absorption of the reaction products was determined in water and the  $\lambda_{max}$  (nm) for the absorbances is also reported in Table 1.

TABLE 1

| Reaction Product | Cyclodiazia-compound (M1) | Epoxide-containing compound (M2) | Monomer 3 (M3) | Molar ratio M1:M2:M3 | $\lambda_{max}$ (nm) |
|------------------|---------------------------|----------------------------------|----------------|----------------------|----------------------|
| 1                |                           |                                  |                | 1:0.63               | 217                  |
| 2                |                           |                                  |                | 1:0.63               | 232                  |

TABLE 1-continued

| Reaction Product | Cyclodiaz-a-compound (M1)                                                           | Epoxide-containing compound (M2)                                                                | Monomer 3 (M3)                                                                        | Molar ratio M1:M2:M3 | $\lambda_{max}$ (nm) |
|------------------|-------------------------------------------------------------------------------------|-------------------------------------------------------------------------------------------------|---------------------------------------------------------------------------------------|----------------------|----------------------|
| 3                |    |               |                                                                                       | 1:0.63               | 220                  |
| 4                |    |               |                                                                                       | 1:0.63               | 222                  |
| 5                |    |               |                                                                                       | 1:0.63               | 207, 263, 273, 292   |
| 6                |    |                |                                                                                       | 1:0.63               | 223                  |
| 7                |   |               |                                                                                       | 1:0.63               | 223                  |
| 8                |  |              |                                                                                       | 1:0.63               | 223                  |
| 9                |  |              |                                                                                       | 1:1                  | 226                  |
| 10               |  |              |                                                                                       | 1:1                  | 222                  |
| 11               |  | <br>Mw = 526 |                                                                                       | 1:0.63               | 234                  |
| 12               |  |             |  | 1:2.65:3             | 196, 250             |

TABLE 1-continued

| Reaction Product | Cyclodiaz-a-compound (M1) | Epoxide-containing compound (M2) | Monomer 3 (M3) | Molar ratio M1:M2:M3 | $\lambda_{max}$ (nm) |
|------------------|---------------------------|----------------------------------|----------------|----------------------|----------------------|
| 13               |                           |                                  |                | 1:2.65:3             | 203, 251             |
| 14               |                           |                                  |                | 1:2.65:3             | 251                  |
| 15               |                           |                                  |                | 1:2.65:3             | 197, 251             |
| 16               |                           |                                  |                | 1:0.63               | 220                  |
| 17               |                           |                                  |                | 1:0.63               | 210, 238, 372        |
| 18               |                           |                                  |                | 1:0.63               | 214, 324             |

**21**  
EXAMPLE 4

**22**

The general procedures of Examples 1 or 2 are repeated except that the following cyclodiazia-compounds and epoxide-containing monomers are used in the ratios listed in Table 2.

TABLE 2

| Reaction Product | Cyclodiazia-compound (M1) | Epoxide-containing compound (M2) | Monomer 3 (M3) | Molar ratio M1:M2:M3 |
|------------------|---------------------------|----------------------------------|----------------|----------------------|
| 20               |                           |                                  |                | 1:2.75:3             |
| 21               |                           |                                  |                | 1:0.65               |
| 22               |                           |                                  |                | 1:1.33:1             |
| 23               |                           |                                  |                | 1:0.7                |
| 24               |                           |                                  |                | 1:0.63               |
| 25               |                           |                                  |                | 1:0.42:0.21          |
| 26               |                           |                                  |                | 1:0.65               |
| 27               |                           |                                  |                | 1:0.33:0.32          |

TABLE 2-continued

| Reaction Product | Cyclodiazia-compound (M1)                                                         | Epoxide-containing compound (M2)                                                  | Monomer 3 (M3) | Molar ratio M1:M2:M3 |
|------------------|-----------------------------------------------------------------------------------|-----------------------------------------------------------------------------------|----------------|----------------------|
| 28               |  |  |                | 1:0.7                |

## EXAMPLE 5

A copper plating bath was prepared by combining 75 g/L copper as copper sulfate pentahydrate, 240 g/L sulfuric acid, 60 ppm chloride ion, 1 ppm of an accelerator and 1.5 g/L of a suppressor. The accelerator was a disulfide compound having sulfonic acid groups and a molecular weight of <1000. The suppressor was an EO/PO copolymer having a molecular weight of <5,000 and terminal hydroxyl groups. The plating bath also contained 3 mL/L of a stock solution of the reaction product from Example 1.

## EXAMPLE 6

Various copper plating baths were prepared generally according to Example 5, except that each of the reaction products of Examples 2-3 were used in the amount of 0.2-4.0 mL/L.

## EXAMPLE 7

Samples (either 3.2 mm or 1.6 mm thick) of a double-sided FR4PCB (5×9.5 cm) having through-holes were plated in a Haring cell using copper plating baths according to Example 4. The 3.2 mm thick samples had 0.3 mm diameter through-holes and the 1.6 mm thick samples had 0.25 mm diameter through-holes. The temperature of each bath was 25° C. A current density of 2.16 A/dm<sup>2</sup> (20 A/ft<sup>2</sup>) was applied to the 3.2 mm samples for 80 minutes and a current density of 3.24 A/dm<sup>2</sup> (30 A/ft<sup>2</sup>) was applied to the 1.6 mm samples for 44 minutes. The copper plated samples were analyzed to determine the throwing power ("TP") of the plating bath, extent of nodule formation, and percent cracking according to the following methods. The amount of the accelerator in each plating bath was 1 ppm. The amount of the leveling agent used in each plating bath and the plating data are shown in Table 3.

Throwing power was calculated by determining the ratio of the average thickness of the metal plated in the center of a through-hole compared to the average thickness of the metal plated at the surface of the PCB sample and is reported in Table 3 as a percentage.

Nodule formation was determined both by visual inspection and by using the Reddington Tactile Test ("RTT"). Visual inspection showed the presence of nodules while the RTT was used to determine the number of nodules. The RTT employs a person's finger to feel the number of nodules for a given area of the plated surface, which in this example was both sides of the PCB sample (total area of 95 cm<sup>2</sup>).

The percent cracking was determined according to the industry standard procedure, IPC-TM-650-2.6.8. Thermal Stress, Plated-Through Holes, published by IPC (Northbrook, Ill., USA), dated May, 2004, revision E.

Plating bath performance was evaluated by throwing power, number of nodules and cracking. The higher the throwing power (preferably ≥70%), the lower the number of

nodules and the lower the percentage of cracking, the better the plating bath performed. As can be seen from the data, plating bath performance can be easily adjusted by increasing or decreasing the amount of the leveling agent in the plating bath.

TABLE 3

| Reaction Product | ppm | TP (%) | Nodules | Cracking (%) |
|------------------|-----|--------|---------|--------------|
| 1                | 1   | 70     | 0       | 0            |
|                  | 5   | 73     | 2       | 0            |
| 2                | 1   | 78     | 0       | 0            |
|                  | 10  | 81     | "       | 0            |
|                  | 20  | 78     | "       | 0            |
| 3                | 1   | 74     | 0       | 0            |
|                  | 5   | 77     | "       | 0            |
|                  | 20  | 83     | "       | 0            |
| 4                | 1   | 71     | 0       | 0            |
|                  | 10  | 80     | 2       | 0            |
|                  | 20  | 83     | 5       | 0            |
| 5                | 1   | 80     | 0       | 0            |
|                  | 5   | 86     | "       | 63           |
|                  | 10  | 81     | 4       | 100          |
|                  | 20  | 75     | 18      | 94           |
| 6                | 1   | 65     | 0       | 0            |
|                  | 5   | 69     | 0       | 0            |
|                  | 10  | 66     | 40      | 0            |
|                  | 20  | 71     | 11      | 0            |
| 7                | 1   | 70     | 0       | 0            |
|                  | 5   | 85     | 1       | 0            |
|                  | 10  | 86     | 60      | 0            |
|                  | 20  | 79     | 45      | 0            |
| 8                | 1   | 74     | 0       | 0            |
|                  | 5   | 75     | "       | 0            |
|                  | 10  | 76     | 20      | 0            |
|                  | 20  | 85     | 10      | 0            |
| 9                | 1   | 68     | 0       | 0            |
|                  | 5   | 54     | "       | 0            |
|                  | 20  | 74     | 2       | 0            |
| 10               | 1   | 60     | 0       | 0            |
|                  | 5   | 70     | "       | 0            |
|                  | 20  | 73     | "       | 0            |
| 11               | 1   | 73     | 0       | 0            |
|                  | 5   | 89     | "       | 0            |
|                  | 20  | 89     | "       | 0            |
| 12               | 1   | 76     | 0       | 0            |
|                  | 5   | 83     | "       | 0            |
|                  | 20  | 90     | "       | 93           |
| 13               | 1   | 78     | 0       | 0            |
|                  | 5   | 90     | "       | 0            |
|                  | 20  | 88     | "       | 0            |
| 14               | 5   | 72     | 1       | 0            |
|                  | 20  | 86     | 25      | 0            |
| 15               | 1   | 82     | 0       | 0            |
| 16               | 1   | 63     | 0       | 0            |
|                  | 5   | 57     | 0       | 0            |
|                  | 10  | 73     | 3       | 0            |
|                  | 20  | 70     | 0       | 0            |
| 17               | 1   | 69     | 0       | 0            |
|                  | 5   | 68     | 9       | 100          |
|                  | 10  | 61     | 25      | 100          |
| 18               | 1   | 60     | 0       | 0            |

TABLE 3-continued

| Reaction Product | ppm | TP (%) | Nodules | Cracking (%) |
|------------------|-----|--------|---------|--------------|
| 19               | 10  | 72     | 3       | 0            |
|                  | 20  | 69     | 0       | 0            |
|                  | 1   | 76     | 0       | 0            |
|                  | 5   | 71     | 0       | 0            |
|                  | 10  | 75     | 2       | 0            |

What is claimed is:

1. A copper electroplating bath comprising: a source of copper ions, an acid electrolyte, an accelerator, and a leveling agent, wherein the accelerator comprises one or more sulfur atoms and has a molecular weight of 1000 or less, and wherein the leveling agent is a reaction product of one or more cyclodiazia-compounds with one or more epoxide-containing compounds; wherein at least one cyclodiazia-compound has the formula (I)



(I)

wherein E=C(O) or CR<sup>5</sup>R<sup>6</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>2</sup> and R<sup>3</sup>, R<sup>3</sup> and R<sup>4</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring; wherein the electroplating bath is acidic.

2. The copper electroplating bath of claim 1 wherein the epoxide-containing compound comprises from 1 to 3 epoxy groups.

3. The copper electroplating bath of claim 2 wherein the epoxide-containing compound is chosen from compounds of the formulae



where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>)alk-

enyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>11</sup>=(CR<sup>13</sup>R<sup>14</sup>)<sub>m</sub>O<sub>n</sub>, (aryl-O)<sub>p</sub>, CR<sup>13</sup>R<sup>14</sup>-Z-CR<sup>13</sup>R<sup>14</sup>O or OZ<sup>1</sup>O; R<sup>12</sup>=(CH<sub>2</sub>)<sub>y</sub>; A1 is a (C<sub>5</sub>-C<sub>12</sub>)cycloalkyl ring or a 5- to 6-membered cyclic-sulfone ring; Z=a 5- or 6-membered ring; Z<sup>1</sup> is R<sup>15</sup>OArOR<sup>15</sup>, (R<sup>16</sup>O)<sub>a</sub>Ar(OR<sup>16</sup>)<sub>a</sub>, or (R<sup>16</sup>O)<sub>a</sub>Cy(OR<sup>16</sup>)<sub>a</sub>; Z<sup>2</sup>=SO<sub>2</sub> or



Cy=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>)alkyl; each R<sup>16</sup> represents a (C<sub>2</sub>-C<sub>6</sub>)alkyleneoxy; each a=1-10; m=1-6; n=1-20; p=1-6; t=1-4; v=0-3; and y=0-6; wherein Y<sup>1</sup> and Y<sup>2</sup> may be taken together to form a (C<sub>8</sub>-C<sub>12</sub>)cyclic compound.

4. The copper electroplating bath of claim 1 wherein at least one of the cyclodiazia-compounds of formula (I) has the formulae (IIa) or (IIb)



(IIa)



(IIb)

wherein R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>4</sup> and R<sup>7</sup> to R<sup>10</sup> are independently chosen from H, (C<sub>1</sub>-C<sub>6</sub>)alkyl, (C<sub>6</sub>-C<sub>10</sub>)aryl and hydroxyl; R<sup>7</sup> and R<sup>9</sup> may be taken together to form a chemical bond; and any of R<sup>1</sup>, R<sup>4</sup> and R<sup>7</sup> to R<sup>10</sup> on adjacent ring atoms may be taken together along with the atoms to which they are attached to form a 5- or 6-membered saturated or unsaturated ring.

5. The copper electroplating bath of claim 4 wherein at least one of the cyclodiazia-compounds is chosen from pyrazole, 3-methylpyrazole, 4-methylpyrazole, 3,4-dimethylpyrazole, 3,5-dimethylpyrazole, 3-phenylpyrazole, 3,5-diphenylpyrazole, 3-(2-hydroxyphenyl)pyrazole, indazole, 4,5,6,7-tetrahydroindazole, 3-methyl-3-pyrazolin-5-one, 4-methyl-2-pyrazolin-5-one, 1-phenyl-3-pyrazolidinone, and 1-phenyl-4,4-dimethyl-3-pyrazolidinone.

6. The copper electroplating bath of claim 1 wherein at least one of the cyclodiazia-compounds of formula (I) has the formulae (IIIa) or (IIIb)



(IIIa)

60

27

-continued



(IIIb)

wherein R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>4</sup> and R<sup>5</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> and R<sup>5</sup> to R<sup>10</sup> on adjacent ring atoms may be taken together along with the atoms to which they are attached to form a 5- or 6-membered saturated or unsaturated ring.

7. The copper electroplating bath of claim 6 wherein at least one of the cyclodiazia-compounds is chosen from pyridazine, 3-methylpyridazine, 4-methylpyridazine, 3,6-dihydroxypyridazine, 3,6-dihydroxy-4-methyl-pyridazine, phthalazine, 6-phenyl-3(2H)-pyridazinone, 6-(2-hydroxyphenyl)-3(2H)-pyridazinone, 4,5-dihydro-6-phenyl-3(2H)-pyridazinone, 1(2H)-phthalazinone, 4-phenylphthalazin-1(2H)-one, 4-(4-methylphenyl)phthalazin-1(2H)-one, and 4-(4-chlorophenyl)phthalazin-1(2H)-one.

8. The copper electroplating bath of claim 1 wherein the accelerator comprises sulfide and/or sulfonic acid groups.

9. The copper electroplating bath of claim 1 wherein the accelerator comprises a moiety of the formula R'-S—R—SO<sub>3</sub>X, where R is optionally substituted alkyl, optionally substituted heteroalkyl, optionally substituted aryl, or optionally substituted heterocyclic; X is a counter ion; and R' is hydrogen or a chemical bond.

10. A method of depositing copper on a substrate comprising: contacting a substrate to be plated with copper with an acidic copper electroplating bath comprising: a source of copper ions, an acid electrolyte, an accelerator, and a leveling agent, wherein the accelerator comprises one or more sulfur atoms and has a molecular weight of 1000 or less, and wherein the leveling agent is a reaction product of one or more cyclodiazia-compounds with one or more epoxide-containing compounds; wherein at least one cyclodiazia-compound has the formula (I)



(I)

28

wherein E=C(O) or CR<sup>3</sup>R<sup>4</sup>; G=CR<sup>5</sup>R<sup>6</sup> or a chemical bond; R<sup>1</sup> and R<sup>2</sup> are independently chosen from H, (C<sub>1</sub>-C<sub>6</sub>)alkyl and (C<sub>6</sub>-C<sub>10</sub>)aryl; R<sup>3</sup> to R<sup>10</sup> are independently chosen from H, (C<sub>1</sub>-C<sub>6</sub>)alkyl, (C<sub>6</sub>-C<sub>10</sub>)aryl and hydroxyl; each of R<sup>1</sup> and R<sup>2</sup>, R<sup>5</sup> and R<sup>7</sup>, R<sup>7</sup> and R<sup>9</sup>, and R<sup>9</sup> and R<sup>1</sup> may be taken together to form a chemical bond; and any of R<sup>1</sup> to R<sup>10</sup> on adjacent ring atoms may be taken together along with the atoms to which they are attached to form a 5- or 6-membered saturated or unsaturated ring; and applying a current density for a period of time sufficient to deposit a copper layer on the substrate.

11. The method of claim 10 wherein the epoxide-containing compound is chosen from compounds of the formulae



where Y, Y<sup>1</sup> and Y<sup>2</sup> are independently chosen from H and (C<sub>1</sub>-C<sub>4</sub>)alkyl; each Y<sup>3</sup> is independently chosen from H, an epoxy group, and (C<sub>1</sub>-C<sub>6</sub>)alkyl; X=CH<sub>2</sub>X<sup>2</sup> or (C<sub>2</sub>-C<sub>6</sub>)alkenyl; X<sup>1</sup>=H or (C<sub>1</sub>-C<sub>5</sub>)alkyl; X<sup>2</sup>=halogen, O(C<sub>1</sub>-C<sub>3</sub>)alkyl or O(C<sub>1</sub>-C<sub>3</sub>)haloalkyl; A=OR<sup>11</sup> or R<sup>12</sup>; R<sup>11</sup>=(CR<sup>13</sup>R<sup>14</sup>)<sub>m</sub>O<sub>a</sub>, (aryl-O)<sub>p</sub>, CR<sup>13</sup>R<sup>14</sup>—Z—CR<sup>13</sup>R<sup>14</sup>O or OZ<sup>1</sup>O; R<sup>12</sup>=(CH<sub>2</sub>)<sub>t</sub>; A1 is a (C<sub>5</sub>-C<sub>12</sub>)cycloalkyl ring or a 5- to 6-membered cyclic-sulfone ring; Z= a 5- or 6-membered ring; Z<sup>1</sup> is R<sup>15</sup>OArOR<sup>15</sup>, (R<sup>16</sup>O)<sub>a</sub>Ar(OR<sup>16</sup>)<sub>a</sub> or (R<sup>16</sup>O)<sub>a</sub>Cy(OR<sup>16</sup>)<sub>a</sub>; Z<sup>2</sup>=SO<sub>2</sub> or

45 (I)

50 Cy=(C<sub>5</sub>-C<sub>12</sub>)cycloalkyl; each R<sup>13</sup> and R<sup>14</sup> are independently chosen from H, CH<sub>3</sub> and OH; each R<sup>15</sup> represents (C<sub>1</sub>-C<sub>8</sub>) alkyl; each R<sup>16</sup> represents a (C<sub>2</sub>-C<sub>6</sub>)alkyleneoxy; each a=1-10; m=1-6; n=1-20; p=1-6; t=1-4; v=0-3; and y=0-6; 55 wherein Y<sup>1</sup> and Y<sup>2</sup> may be taken together to form a (C<sub>8</sub>-C<sub>12</sub>) cyclic compound.

\* \* \* \* \*